

## UNITED STATES PATENT OFFICE.

WILLIAM PORTER DREAPER, OF HAMPSTEAD HEATH, LONDON, ENGLAND.

## MANUFACTURE OF ARTIFICIAL SILK AND THE LIKE FROM VISCOSE SOLUTIONS.

No Drawing. Application filed August 31, 1925, Serial No. 53,748, and in Great Britain September 17, 1924.

This invention relates to an improved process for the production of artificial yarn of the kind in which the filaments are dried in the skein form under tension in the gel condition so as to cause them to adhere temporarily to each other in such a manner as to resemble what is known as "raw" or "gum" natural silk, and my said invention has for its object to produce such artificial "gum" silk yarns from viscose solution.

In the treatment of viscose artificial silk it is necessary to remove the sulphur from the freshly spun filaments. This treatment has heretofore taken place after the filaments have been washed and dried under tension on a stretching frame so that they are no longer in a gel condition, since it has been found that the desulphurizing solution consisting e. g. of sodium sulphide with possibly some free caustic soda in it, is liable to increase the hydration of the freshly spun filaments and thereby reduce their mechanical strength so that it is not practicable to desulphurize them and then dry them under tension whilst still in the gel condition.

According to my invention, in order to enable the filaments to be desulphurized or if desired desulphurized and bleached, or both bleached and dyed, in the gel condition and then dried under tension, the freshly precipitated gel filaments, before they are dried, are treated with a desulphurizing solution to which there is added not less than 40 per cent of the saturation value at normal atmospheric temperatures of a suitable salt or salts (i. e. any soluble salt other than the sulphide) of an alkali metal or metals (i. e. sodium, potassium, or ammonium). For example, sufficient common salt is added to bring the concentration of the bath up to 80 per cent of its saturation value in respect to such salt. With concentrations of salt substantially less than the 40 per cent above mentioned, the filaments are unable to withstand the tension necessary to be applied during drying. It is an advantage to make a similar addition of a salt or salts of an alkali metal or metals to the dyeing, bleaching and other baths through which the threads desulphurized as above described are subsequently passed. When such an addition is made it is not necessary, owing to the relatively milder condi-

tions obtaining in the treatment, to add such a large proportion of salt. In some cases a proportion as low as 10 per cent of the saturation limit is found to give beneficial results. Moreover e. g. in cases where the dyeing takes place in a sodium sulphide solution, the desulphurizing and dyeing may take place simultaneously, provided the dyeing action be not prevented by the salting out of the dye stuff.

By this means, the filaments are prevented from being further hydrated during their exposure to the action of the desulphurizing and other (e. g. bleaching or dyeing) baths, and thus their mechanical strength is preserved or even increased so as to enable them to be dried under tension in the gel condition in order to produce artificial silk of the "gum" type having the filaments adhering together.

Also while the filaments are still in the gel condition and ready to be immersed in the final wash water, which may or may not contain added soluble salts, this water may have added to it a suitable sizing material such as for instance a small amount of soluble starch, but in this case the wash water, or solution used for the final treatment of the yarn after it has been dried and worked up, must be of such a nature or temperature or both as to enable it to remove the added dressing material or size.

By the means explained a viscose product can be obtained which very closely resembles "raw" silk, and this is found to be of particular advantage where fine denier yarns consisting of fine denier filaments are required. There is also a saving in the cost of producing the artificial silk yarn by obviating the necessity for the second drying of the filaments which normally takes place in the processes of manufacture heretofore adopted. The risk of damage to the filaments resultant upon the handling operations necessary to such second drying is thus eliminated.

I claim:

1. A process of producing artificial filaments and yarns in imitation of "gum type" silk wherein the freshly precipitated gel filaments produce from viscose solutions, before they are dried in a state of tension, are treated with a desulphurizing solution to which there is added alkali metal salt in

amount not less than 40 per cent of the saturation value at normal atmospheric temperatures.

2. A process of producing artificial filaments and yarns in imitation of "gum type" silk wherein the freshly precipitated gel filaments produced from viscose solutions, before they are dried in a state of tension, are treated with a desulphurizing solution to which there is added common salt in amount not less than 40 per cent of the saturation value at normal atmospheric temperatures.

3. A process of producing artificial filaments and yarns in imitation of "gum type" silk wherein the freshly precipitated gel filaments produced from viscose solutions, before they are dried in a state of tension, are treated with a desulphurizing solution to which there is added common salt

the amount of which is substantially 80 per cent of the saturation value at normal atmospheric temperatures.

4. A process of producing artificial filaments and yarns in imitation of "gum type" silk wherein the freshly precipitated gel filaments produced from viscose solutions, before they are dried in a state of tension, are treated with a desulphurizing solution to which there is added suitable alkali metal salt in amount not less than 40 per cent of the saturation value at normal atmospheric temperatures, suitable salt of an alkali metal being also added but in a smaller proportion to baths which are additional to the desulphurizing bath and with which the filaments are treated whilst still in a gel condition.

WILLIAM PORTER DREAPER.